



US005411841A

**United States Patent** [19]

Singer et al.

[11] **Patent Number:** **5,411,841**[45] **Date of Patent:** **May 2, 1995**[54] **PHOTOGRAPHIC ELEMENTS  
CONTAINING MAGENTA COUPLERS AND  
PROCESS FOR USING SAME**[75] Inventors: **Stephen P. Singer**, Spencerport; **Paul B. Merkel**, Rochester, both of N.Y.; **Bernard A. J. Clark**, Berkshire; **Paul L. R. Stanley**, Harrow, both of United Kingdom[73] Assignee: **Eastman Kodak Company**, Rochester, N.Y.[21] Appl. No.: **66,960**[22] Filed: **May 24, 1993**[51] Int. Cl.<sup>6</sup> ..... **G03C 7/384**[52] U.S. Cl. ..... **430/387; 430/555**[58] Field of Search ..... **430/555, 387**[56] **References Cited****U.S. PATENT DOCUMENTS**

- 4,463,085 7/1984 Mitsui ..... 430/372  
4,483,918 11/1984 Sakai et al. ..... 430/372  
4,555,479 11/1985 Sakai et al. ..... 430/372  
4,853,319 8/1989 Krishnamurthy et al. ..... 430/387  
4,900,657 2/1990 Crawley et al. ..... 430/555  
4,904,579 2/1990 Mihayashi et al. ..... 430/551  
4,952,487 8/1990 Renner et al. ..... 430/546  
4,994,359 2/1991 Moriyuki et al. ..... 430/555  
5,250,407 10/1993 Kase ..... 430/555

**FOREIGN PATENT DOCUMENTS**

- 0002953 1/1985 Japan ..... 430/555  
1494777 12/1977 United Kingdom .  
2244053 11/1991 United Kingdom .

*Primary Examiner*—Lee C. Wright*Attorney, Agent, or Firm*—Arthur E. Kluegel[57] **ABSTRACT**

Improved hue, speed of dye formation and reduced

staining are provided by a photographic element comprising a light-sensitive silver halide layer having associated therewith a 1-phenyl-3-anilino-pyrazolo-5-one coupler comprising a ballasted parent and a coupling-off group and containing substituents on the 1-phenyl and 3-anilino rings of the parent having Hammett sigma values which together sum to at least 1.1, the coupler further having at the 4-position of the pyrazolone ring a coupling-off group comprising a phenylthio group containing a carbonamido substituent in the position para to the sulfur on the phenylthio ring with the substituents on the phenylthio ring selected such that the calculated log P of the thiophenol corresponding to the coupling-off group is at least 4.

Example coupler:

**8 Claims, No Drawings**

PHOTOGRAPHIC ELEMENTS CONTAINING  
MAGENTA COUPLERS AND PROCESS FOR  
USING SAME

FIELD OF THE INVENTION

This invention relates to photographic elements containing magenta couplers comprising a parent 1-phenyl-3-anilino-pyrazolo-5-one and a phenylthio coupling-off group with both the parent and coupling-off group containing substituents providing improved hue, speed of dye formation and reduced staining.

BACKGROUND OF THE INVENTION

The use of magenta couplers comprising 1-phenyl-3-anilino-pyrazolo-5-one couplers containing phenylthio coupling-off groups at the 4-position are well known in the art. See for example U.S. Pat. No. 4,853,319 of Krishnamurthy et al. and other patents cited therein. While elements employing such couplers have provided certain advantages, there remain several shortcomings in photographic elements relying on these types of magenta couplers.

These shortcomings relate to the dye-forming efficiency of the coupler, the speed with which the dye is formed, the dye hue, and the undesirable occurrence of staining during processing. Compositions disclosed in the mentioned U.S. Pat. No. 4,853,319 contain an ortho carbonamido substituent on the phenylthio coupling-off group of the magenta coupler. It has been found that compounds of this type provide disadvantages in terms of the speed of dye formation and staining.

The dye forming efficiency of the coupler is affected by many factors such as the extent to which the parent portion of the coupler is ballasted so as to retain its proper position in the photographic element in order to optimize the image recorded. If the coupler parent is not sufficiently ballasted, it is free to wander both horizontally and vertically during processing thereby adversely affecting both sharpness and color rendition. Moreover, the coupler is susceptible to being washed out of the element entirely and thus contributing no dye density to the image. Therefore, this problem is to be avoided.

The dye efficiency can also be affected by the coupling-off group. If the coupling-off group is able to migrate upon release and if it is capable of interfering in the desired chain of reactions that allows the reduction of silver to transform a corresponding amount of coupler to dye, then the coupling-off group can itself cause a reduction in dye formation efficiency.

The speed with which the dye is formed can present added problems. When a coupler undergoes coupling with a color developer to form a dye, the coupler goes through an intermediate stage wherein the oxidized developer and the coupling-off group are both annexed to the coupler parent. This intermediate is a leuco dye which is uncolored until the coupling reaction is complete. In the ideal photographic element, the intermediate stage is essentially instantaneous so that the process of dye formation is completed during development. The presence of the semi-stable leuco dye can effectively reduce dye density and adversely affect color rendition in the printing step. Moreover the presence of the semi-stable leuco dye can lead to post processing density increases the extent of which cannot be predicted and this leads to the undesirable situation of having an image

which changes with time. Thus, the formation of semi-stable leuco dyes needs to be avoided.

Of further concern is the hue of the dye obtained upon completion of the coupling reaction. This property is important because it affects the accuracy of color rendition and also impacts the printer's ability to produce an accurate print from the negative. The hue of the dye is a function of the compositional make-up of both the parent and the coupling-off group. Both the individual substituents and the combined effect of the different substituents selected can affect the hue. The parent substituents affect hue primarily through their effect on the chromophore of the dye while the coupling-off group substituents have a more indirect effect by influencing the local environment of the dye, particularly when the coupled-off group is not free to diffuse away from the hydrophobic oil droplet.

Finally, staining or nonimagewise coloration of the element is to be avoided. One way that staining can occur is through the phenomenon called continued coupling. Certain couplers are more prone than others to react with oxidized developer that is carried over with the film into the bleach bath. These couplers will thus form dye on a non-imagewise basis causing a magenta stain.

While various efforts have been made to provide improved couplers, none have succeeded in solving the foregoing problems.

U.S. Pat. Nos. 4,555,479; 4,463,085; 4,483,918; and 4,904,579, all deal with the suggestion of various additives to elements containing 1-phenyl-3-anilino-pyrazolo-5-one couplers containing phenylthio or other types of coupling-off groups at the 4-position in order to improve sensitivity, stability etc. The materials exemplified therein do not provide the desired properties such as diffusion resistance of both the parent and coupling-off group. U.K. Patent 1,494,777 suggests couplers having improved properties such as high dye yield without formation of undesirable fog and stain. The couplers therein are unsatisfactory since the formed dyes are either not sufficiently ballasted to prevent washout during processing or do not exhibit the improvements specified herein.

U.S. Pat. No. 4,952,487 relates to the use of alkyl-phenol coupler solvents for hue improvement and suggests certain elements containing 1-phenyl-3-anilino-pyrazolo-5-one couplers containing phenylthio or other types of coupling-off groups at the 4-position. These couplers do not, however, solve the problems mentioned since efficiency is adversely affected by the coupling-off groups present.

It is therefore a problem to be solved to provide photographic elements containing a magenta coupler which does not present problems associated with the dye-forming efficiency of the coupler, the speed with which the dye is formed, the dye hue, and the undesirable occurrence of staining during processing.

SUMMARY OF THE INVENTION

The invention provides a photographic element comprising a light-sensitive silver halide layer having associated therewith a 1-phenyl-3-anilino-pyrazolo-5-one coupler comprising a ballasted parent and a coupling-off group and containing substituents on the 1-phenyl and 3-anilino rings of the parent having Hammett sigma values which together sum to at least 1.1, the coupler further having at the 4-position of the pyrazolone ring a coupling-off group comprising a phenylthio group con-

taining a carbonamido substituent in the position para to the sulfur on the phenylthio ring with the substituents on the phenylthio ring selected such that the calculated log P of the thiophenol corresponding to the coupling-off group is at least 4.

The invention also provides a process for forming images from an exposed element of the type described above through development employing a color development chemical.

The element and process of the invention provide improved photographic properties such as those relating to the dye-forming efficiency of the coupler, the speed with which the dye is formed, the dye hue, and the undesirable occurrence of staining during processing.

#### DETAILED DESCRIPTION OF THE INVENTION

The invention provides a photographic element comprising a light-sensitive silver halide layer having associated therewith a 1-phenyl-3-anilino-pyrazolo-5-one coupler comprising a ballasted parent and a coupling-off group and containing substituents on the 1-phenyl and 3-anilino rings of the parent having Hammett sigma values which together sum to at least 1.1, said coupler further having at the 4-position of the pyrazolone ring a coupling-off group comprising a phenylthio group containing a carbonamido substituent in the position para to the sulfur on the phenylthio ring with the substituents on the phenylthio ring selected such that the calculated log P of the thiophenol corresponding to the coupling-off group is at least 4.

A photographic element of the invention comprises a light-sensitive silver halide layer having associated therewith a coupler which is a pyrazolone compound containing a phenyl and an anilino substituent and having formula I:



wherein:

each R<sup>1</sup> is independently a substituent provided that the sum of the Hammett sigma values for all R<sup>1</sup> groups is at least 1.1 and the combined R<sup>1</sup> substituents are sufficient to ballast the dye formed by the parent upon coupling;

R<sup>2</sup> is hydrogen or alkyl of up to two carbon atoms;

R<sup>3</sup>, when present, is a substituent (preferably substituted or unsubstituted alkyl of up to 24 carbon atoms); R<sup>4</sup> is a substituted or unsubstituted alkyl or aryl group; R<sup>5</sup> is hydrogen or substituted or unsubstituted alkyl; X is —O— or —N(R<sup>6</sup>) wherein R<sup>6</sup> is

hydrogen or alkyl; m is 0 or 1; n1 and n2 are 0 to 5; p is 0 to 3;

provided that any combination of R<sup>3</sup>, R<sup>4</sup>, and R<sup>5</sup> may join together to form a ring; and

provided further that each of R<sup>2</sup> through R<sup>6</sup> along with X and m are selected such that the calculated log P of the thiophenol corresponding to the substituent at the 4-position of the pyrazolone is at least 4.

In a more preferred embodiment, the coupler has formula II:



wherein:

R<sup>a</sup> is located in the 4- or 5-position of the anilino ring and is a substituent selected from those which are attached to the anilino ring by a member selected from the group consisting of —SO—; —SO<sub>2</sub>—; —OSO<sub>2</sub>—; —SO<sub>2</sub>N<; >NSO<sub>2</sub>—; —CON<; >NCO—; —CO—; —OCO—; —COO—; —CN; —NO<sub>2</sub>; and —CF<sub>3</sub>;

each R<sup>c</sup> is individually halogen, or substituted or unsubstituted alkyl (such as trifluoromethyl), aryl-oxo or alkoxy;

each R<sup>b</sup> is individually hydrogen or a substituent selected so that the sum of the Hammett sigma values for all R<sup>a</sup>, R<sup>b</sup>, and R<sup>c</sup> groups is at least 1.1 and the combination of such substituents is sufficient to ballast the dye formed upon coupling;

q is 0 to 3, and r is 0 to 2; R<sup>2</sup> is hydrogen or alkyl of up to two carbon atoms; each R<sup>3</sup>, when present, is independently a substituent, preferably an alkyl substituent of up to 24 carbon atoms; R<sup>4</sup> is a substituted or unsubstituted alkyl or aryl group; R<sup>5</sup> is hydrogen or substituted or unsubstituted alkyl; p is 0 to 3;

provided that any combination of R<sup>3</sup>, R<sup>4</sup>, and R<sup>5</sup> may join together to form a ring; and

provided further that each of R<sup>2</sup> through R<sup>5</sup> are selected such that the calculated log P of the thiophenol corresponding to the substituent at the 4-position of the pyrazolone is at least 4.

The parent group of the coupler contains substituents sufficient to ballast the dye formed by the parent upon coupling. Ballast groups are well-known in the art. Desirably a ballasted coupler contains sufficient hydrophobic groups to prevent it from migrating from the organic phase during processing. Otherwise, it may wash out as coupler or dye and will not contribute to desired dye density. This will be seen as a loss in dye forming efficiency. Preferably, the coupler contains at

least 7 and most preferably at least 10 alkyl carbon atoms in order to provide the desired degree of ballasting.

Hammett sigma values are well known in the art as a measure of the relative electron withdrawing or electron donating effect that a particular substituent has on a ring or group to which it is attached. By convention, hydrogen has a sigma value of 0 with positive sigma values indicating more electron withdrawing power than hydrogen, and negative values indicating more electron donating effect than hydrogen. Values for sigma were found in published chemical literature (see for example "The Chemist's Companion", A. J. Gordon and R. A. Ford, John Wiley & Sons, New York, 1972; "Progress in Physical Organic Chemistry, Volume 13", R. W. Taft, Ed., John Wiley & Sons, New York; and C. Hansch and A. J. Leo, in "Substituent Constants for Correlation Analysis in Chemistry and Biology", Wiley, New York, 1979). The values for sigma<sub>para</sub> were used to estimate the value for substituents ortho to the pyrazolone nucleus.

The log P referred to herein is the logarithm of the partition coefficient between octanol and water. The photographic element of the invention is a multiphase material and therefore the coupler can distribute itself among the different phases present. The log P indicates the relative solubility of the coupler in the hydrophobic and hydrophilic phases of the element. A compound which partitions equally between the two phases will have a log P of 0. Higher log P values indicate that the compound exhibits increasingly greater hydrophobic properties. Materials with high log P values are essentially confined to the organic phase surrounding the coupler and are not likely to migrate to the hydrophilic gel phase where the light sensitive silver is. This may be particularly important where it is desired to prevent a compound such as a thio coupling-off group from attacking the silver and inhibiting it from developing.

Rather than performing a partition experiment, it is a preferred alternative to calculate the log P of a substituent. The log P values are calculated using the Medchem program, version 3.54, Medicinal Chemistry Project, Pomona College, Claremont Calif. (1984). (For a discussion of this method see Albert J. Leo, in "Comprehensive Medicinal Chemistry", edited by C. Hansch, P. G. Sammes, and J. B. Taylor, Pergamon Press, New York, Volume 4, 1990, and U.S. Pat. No. 4,782,012. ) Values for estimating the log P (or pi) of a substituent are shown in the above mentioned article of C. Hansch and A. J. Leo, in "Substituent Constants for Correlation Analysis in Chemistry and Biology", Wiley, New York, 1979.

The substituents usable for R<sup>1</sup> and, except as otherwise limited, for other indicated substituents herein may be selected from a broad list. They may be, for example, halogen, such as chlorine, bromine or fluorine; nitro; hydroxyl; cyano; carboxyl or its salts; and groups which may be further substituted, such as alkyl, including straight or branched chain alkyl, such as methyl, trifluoromethyl, ethyl, t-butyl, 3-(2,4-di-t-amylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy 2-(2,4-di-t-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolylxy; carbonamido, such as acet-

amido, benzamido, butyramido, tetradecanamido, alpha-(2,4-di-t-pentylphenoxy)acetamido, alpha-(2,4-di-t-pentylphenoxy)butyramido, alpha-(3-pentadecylphenoxy)hexanamido, alpha-(4-hydroxy-3-t-butylphenoxy)tetradecanamido, 2-oxo-pyrrolidin-1-yl, 2-oxo-5-tetradecyl-pyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, 10 phenoxycarbonylamino, benzyloxycarbonylamino, hexadecyloxycarbonylamino, 2,4-di-t-butylphenoxy carbonylamino, phenylcarbonylamino, 2,5-(di-t-pentylphenyl)carbonylamino, p-dodecylphenylcarbonylamino, p-tolylcarbonylamino, N-methylureido, N,N-dimethylureido, N-methyl-N-dodecylureido, N-hexadecylureido, N,N-dioctadecylureido, N,N-dioctyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido; and t-butylcarbonamido; sulfonamido, such as methylsulfonamido, benzenesulfonamido, p-tolylsulfonamido, p-dodecylbenzenesulfonamido, N-methyltetradecylsulfonamido, N,N-dipropylsulfamoylamino, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-dioctylcarbamoyl; acyl, such as acetyl, (2,4-di-t-amylphenoxy)acetyl, phenoxy carbonyl, p-dodecyloxyphenoxy carbonyl methoxycarbonyl, butoxycarbonyl, tetradecyloxycarbonyl, ethoxycarbonyl, benzyloxycarbonyl, 3-pentadecyloxycarbonyl, and dodecyloxycarbonyl; sulfonyl, such as methoxysulfonyl, octyloxysulfonyl, tetradecyloxysulfonyl, 2-ethylhexyloxysulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acetoxy, benzyloxy, octadecanoyloxy, p-dodecylamidobenzoyloxy, N-phenylcarbamoyloxy, N-ethylcarbamoyloxy, and cyclohexylcarbonyloxy; amine, such as phenylanilino, 2-chloroanilino, diethylamine, dodecylamine; imino, such as 1 (N-phenylimido)ethyl, N-succinimido or 3-benzylhydantoinyl; phosphate, such as dimethylphosphate and ethylbutylphosphate; phosphite, such as diethyl and dihexylphosphite; azo, such as phenylazo and naphthylazo; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

The particular substituents used may be selected to attain the desired photographic properties for a specific application and can include, for example, hydrophobic groups, solubilizing groups, blocking groups, etc. Generally, the above groups and substituents thereof may typically include those having 1 to 30 carbon atoms and usually less than 24 carbon atoms, but greater numbers are possible depending on the particular substituents selected. Moreover, as indicated, the substituents may themselves be suitably substituted with any of the above groups. In one embodiment R<sup>1</sup> is an alkyl sulfonyl compound where the alkyl group is 2 to 30 and preferably 2 to 18 carbon atoms.

The R<sup>1</sup> substituents must be selected in a coordinated fashion so that the sum of the Hammett sigma values on the phenyl and anilino rings is at least 1.1. In a preferred embodiment, the sum of the values is at least 1.2 and most preferably at least 1.3. In order to achieve the desired sum it is preferred to select at least one substituent which is attached to the phenyl or anilino ring by a member selected from the group consisting of —SO—; —SO<sub>2</sub>—; —OSO<sub>2</sub>—; —SO<sub>2</sub>N<; >NSO<sub>2</sub>—; —CON<; >NCO—; —CO—; —OCO—; —COO—; —CN; —NO<sub>2</sub>; and —CF<sub>3</sub>.

In the embodiment of formula II, three of the parent substituents, identified as R<sup>c</sup>, are selected from a smaller group as indicated following the formula with chlorine being the most preferred. R<sup>b</sup> may be any suitable substituent and R<sup>a</sup> is a substituent attached to the anilino ring by a member selected from the group consisting of —SO—; —SO<sub>2</sub>—; —OSO<sub>2</sub>—; —SO<sub>2</sub>N<; >NSO<sub>2</sub>—; —CON<; >NCO—; —CO—; —OCO—; —COO—; —CN; —NO<sub>2</sub>; and —CF<sub>3</sub>. In one embodiment R<sup>a</sup> is an alkyl sulfonyl compound where the alkyl group is 2 to 30 and preferably 2 to 18 carbon atoms.

The number of substituents on the parent is not particularly critical so long as the desired sigma sum is attained. "n1" and "n2" may each be 0 to 5 although they cannot both be 0 at the same time. "q" may be 0 to 3 and "r" may be 0 to 2 although they cannot both be 0 at the same time.

The coupling-off group is one comprising a phenylthio group having a certain carbonamido substituent at the 4-position relative to the sulfur. The carbonamido substituent has the general formula “—N(R<sup>5</sup>)-45 C(O)(X)<sub>m</sub>R<sup>4</sup>” where R<sup>4</sup> is a substituted or unsubstituted alkyl or aryl group; R<sup>5</sup> is hydrogen or substituted or unsubstituted alkyl; X is —O— or —N(R<sup>6</sup>) wherein R<sup>6</sup> is hydrogen or alkyl and m is 0 or 1. In a preferred embodiment, the carbonamido has the formula shown 50 in II above where the substituent is a secondary amide (—NHC(O)(X)<sub>m</sub>. The location of the substituent in the 4-position provides advantages in the photographic properties of the coupler compared to alternative locations.

The substituent R<sup>2</sup> on the phenylthio ring should not be too substantial. If not hydrogen, it is preferably an alkyl group of not more than two carbon atoms. R<sup>3</sup> is defined as a substituent chosen from the same group as R<sup>1</sup>, and, when present, is preferably alkyl of up to 24 60 carbon atoms. It may be a broad range of groups and may form a ring with R<sup>4</sup> of the carbonamido group. R<sup>4</sup> may also form a ring with R<sup>5</sup>.

The components R<sup>2</sup> through R<sup>5</sup> must be co-selected so that the calculated log P for the thiophenol corresponding to the coupling-off group is at least 4. This feature helps to limit the diffusability of the group when coupled-off so that there is no interference with the

progress of the desired chain of development reactions. In particular, it helps to prevent the sulfur containing group from attacking and inhibiting the silver being developed. Better results may be obtained in this respect when log P is at least 4.5 or when log P is at least 5.0.

Specific examples of couplers suitable for use in the invention are as follows:



COG =

M-1



M-2





-continued



5,411,841

10

-continued

M-7



5

16

15

M-4

25

30

M-5

40

45

50

55

60



-continued



-continued



25



M-15



M-16

-continued



-continued



15

-continued



The materials of the invention can be used in any of the ways and in any of the combinations in which such compositions are used in the photographic art. Typically, they are incorporated in a silver halide emulsion containing layer and the layer coated on a support to form part of a photographic element. Alternatively, they can be incorporated at a location adjacent to the silver halide emulsion layer where, during development, they will be in reactive association with development products such as oxidized color developing agent. Thus, as used herein, the term "associated" signifies that the coupler is in the silver halide emulsion layer or in an adjacent location where, during processing, the compositions are capable of reacting with silver halide development products. 45 50 55

Representative ballast groups include substituted or unsubstituted alkyl or aryl groups containing 7 to 40 carbon atoms. Representative substituents on such groups include alkyl, aryl, alkoxy, aryloxy, alkylthio, hydroxy, halogen, alkoxy carbonyl, arylox carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 40 carbon atoms. Such substituents can also be further substituted.

The photographic elements can be single color elements or multicolor elements. Multicolor elements con-

M-23

16

tain dye image-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

10 A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

For example, the coupler of the invention may be used to replace all or part of the image coupler or may be added to one or more of the other layers in a color negative photographic element comprising a support bearing the following layers from top to bottom:

- (1) one or more overcoat layers containing ultraviolet absorber(s);

(2) a two-coat yellow pack with a fast yellow layer containing "Coupler 1": Benzoic acid, 4-chloro-3-((2-(4-ethoxy, 2,5-dioxo-3-(phenylmethyl)-1-imidazolidinyl)-3-(4-methoxyphenyl)-1,3-dioxo-propyl)amino)-, dodecyl ester and a slow yellow layer containing the same compound together with "Coupler 2": Propanoic acid, 2-[5-[[4-[2-[[2,4-bis(1,1-dimethylpropyl)phenoxy]acetyl]amino]-5-[(2,2,3,3,4,4,4-heptafluoro-1-oxobutyl) amino]-4-hydroxyphenoxy]-2,3-dihydroxy-6-[(propanoamino)carbonyl ]phenyl]thio]-1,3,4-thiadiazol-2-yl]thio]-, methyl ester and "Coupler 3": 1-((dodecyloxy)carbonyl) ethyl(3-chloro-4-((3-(2-chloro-4-((1-tridecanoylethoxy) carbonyl)anilino)-3-oxo-2-((4)(5)(6)-(phenoxy carbonyl)-1H-benzotriazol-1-yl)propanoyl)amino))benzoate;

(3) an interlayer containing fine metallic silver;

(4) a triple-coat magenta pack with a fast magenta layer containing "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)-, "Coupler 5": Benzamide, 3-((2-(2,4-bis(1,1-dimethylpropyl)phenoxy)-1-oxobutyl)amino)-N-(4', 5'-dihydro-5'-oxo-1'-(2,4,6-trichlorophenyl) (1,4'-bi-1H-pyrazol)-3'-yl)-, "Coupler 6": Carbamic acid, (6-(((3-(dodecyloxy)propyl) amino)carbonyl)-5-hydroxy-1-naphthalenyl)-, 2-methylpropyl ester , "Coupler 7": Acetic acid, ((2-((3-(((3-(dodecyloxy)propyl)amino) carbonyl)-4-hydroxy-8-(((2-methylpropoxy)carbonyl) amino)-1-naphthalenyl)oxy )ethyl)thio)-, and "Coupler 8" Benzamide, 3-((2-(2,4-bis(1,1-dimethylpropyl) phenoxy)-1-oxobutyl)amino)-N-(4,5-dihydro-4-((4-methoxyphenyl) azo)-5-oxo-1-(2,4,6-trichlorophenyl)-1H-pyrazol-3-yl)-; a mid-magenta layer and a slow magenta layer each containing "Coupler 9": a ternary copolymer containing by weight in the ratio 1:1:2 2-Propenoic acid

- butyl ester, styrene, and N-[1-(2,4,6-trichlorophenyl)-4,5-dihydro-5-oxo-1H-pyrazol-3-yl]-2-methyl-2-propenamide; and "Coupler 10": Tetradecanamide, N-(4-chloro-3-((4-((2,2-dimethyl-1-oxopropyl) amino)phenyl)azo)-4,5-dihydro-5-oxo-1-(2,4,6-trichlorophenyl)-1H-pyrazol-3-yl)amino)phenyl)-, in addition to Couplers 3 and 8; 5 (5) an interlayer;
- (6) a triple-coat cyan pack with a fast cyan layer containing Couplers 6 and 7; a mid-cyan containing 10 Coupler 6 and "Coupler 11": 2,7-Naphthalenedisulfonic acid, 5-(acetylamino)-3-((4-(2-((3-(2,4-bis(1,1-dimethylpropyl)phenoxy)-propyl)amino)-carbonyl)-4-hydroxy-1-naphthalenyl)oxy)ethoxy)-phenyl)azo)-4-hydroxy-, disodium salt; and a slow 15 cyan layer containing Couplers 2 and 6;
- (7) an undercoat layer containing Coupler 8; and
- (8) an antihalation layer.

In a color paper format, the coupler of the invention may suitably be used to replace all or a part of the image 20 coupler or added to a layer in a photographic element such as one comprising a support bearing the following from top to bottom:

- (1) one or more overcoats;
- (2) a cyan layer containing "Coupler 1": Butanamide, 25 2-(2,4-bis(1,1-dimethylpropyl)phenoxy)-N-(3,5-dichloro-2-hydroxy-4-methylphenyl), "Coupler 2": Acetamide, 2-(2,4-bis(1,1-dimethylpropyl)phenoxy)-N-(3,5-dichloro-2-hydroxy-4-, and UV Stabilizers: Phenol, 2-(5-chloro-2H-benzotriazol-2-yl)-4,6-bis(1,1-dimethylethyl)-; Phenol, 2-(2H-benzotriazol-2-yl)-4-(1,1-dimethylethyl)-; Phenol, 2-(2H-benzotriazol-2-yl)-  
-(1,1-dimethylethyl)-6-(1-methylpropyl)-; and Phenol, 2-(2H-benzotriazol-2-yl)-4,6-bis(1,1-dimethylpropyl)- and a poly(t-butylacrylamide) dye stabilizer; 35
- (3) an interlayer;
- (4) a magenta layer containing "Coupler 3": Octanamide, 2-[2,4-bis(1,1-dimethylpropyl)phenoxy]-N-[2-(7-chloro-6-methyl-1H-pyrazolo[1,5-b][1,2,4]triazol-2-yl)propyl]- together with 1,1'-Spirobi (1H-indene), 2,2',3,3'-tetrahydro-3,3,3',3'-tetramethyl-5,5',6,6'-tetrapropoxy-; 40
- (5) an interlayer; and
- (6) a yellow layer containing "Coupler 4": 1-Imidazolidineacetamide, N-(5-((2-(2,4-bis(1,1-dimethylpropyl)phenoxy)-1-oxobutyl)amino)-2-chlorophenyl)-.alpha.-(2,2-dimethyl-1-oxopropyl)-4-ethoxy-2,5-dioxo-3-(phenylmethyl)-.

In a reversal medium, the coupler of the invention could be used to replace all or part of the image coupler or added to a layer in a photographic element such as one comprising a support and bearing the following layers from top to bottom:

- (1) one or more overcoat layers;
- (2) a nonsensitized silver halide containing layer;
- (3) a triple-coat yellow layer pack with a fast yellow layer containing "Coupler 1": Benzoic acid, 4-((2-chloro-5-((dodecylsulfonyl)amino)phenyl)amino)carbonyl)-3,3-dimethyl-2-oxobutoxy-, 1-methylethyl ester; a mid yellow layer containing Coupler 1 and "Coupler 2": Benzoic acid, 4-chloro-3-[[2-[4-ethoxy-2,5-dioxo-3-(phenylmethyl)-1-imidazolidinyl]-4,4-dimethyl-1,3-dioxopen-65 tyl]amino]-, dodecylester; and a slow yellow layer also containing Coupler 2;
- (4) an interlayer;

- (5) a layer of fine-grained silver;
- (6) an interlayer;
- (7) a triple-coated magenta pack with a fast magenta layer containing "Coupler 3": 2-Propenoic acid, butyl ester, polymer with N-[1-(2,5-dichlorophenyl)-4,5-dihydro-5-oxo-1H-pyrazol-3-yl]-2-methyl-2-propenamide; "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl); and "Coupler 5": Benzamide, 3-((2,4-bis(1,1-dimethylpropyl)phenoxy)acetyl)amino)-N-(4,5-dihydro-5-oxo-1-(2,4,6-trichlorophenyl)-1H-pyrazol-3-yl); and containing the stabilizer 1,1'-Spirobi(1H-indene), 2,2',3,3'-tetrahydro-3,3,3',3'-tetramethyl-5,5',6,6'-tetrapropoxy-; and in the slow magenta layer Couplers 4 and 5 with the same stabilizer;
- (8) one or more interlayers possibly including fine-grained nonsensitized silver halide;
- (9) a triple-coated cyan pack with a fast cyan layer containing "Coupler 6": Tetradecanamide, 2-(2-cyanophenoxy)-N-(4-((2,2,3,3,4,4,4-heptafluoro-1-oxobutyl)amino)-3-hydroxyphenyl); a mid cyan containing "Coupler 7": Butanamide, N-(4-((2-(2,4-bis(1,1-dimethylpropyl)phenoxy)-1-oxobutyl)amino)-2-hydroxyphenyl)-2,2,3,3,4,4,4-heptafluoro- and "Coupler 8": Hexanamide, 2-(2,4-bis(1,1-dimethylpropyl)phenoxy)-N-(4-(2,2,3,3,4,4,4-heptafluoro-1-oxobutyl)amino)-3-hydroxyphenyl)-;
- (10) one or more interlayers possibly including fine-grained nonsensitized silver halide; and
- (11) an antihalation layer.

If desired, the photographic element can be used in conjunction with an applied magnetic layer as described in *Research Disclosure*, November 1992, Item 34390 published by Kenneth Mason Publications, Ltd., Dudley Annex, 12a North Street, Emsworth, Hampshire PO10 7DQ, ENGLAND.

In the following discussion of suitable materials for use in the emulsions and elements of this invention, reference will be made to *Research Disclosure*, December 1989, Item 308119, available as described above, which will be identified hereafter by the term "Research Disclosure." The contents of the Research Disclosure, including the patents and publications referenced therein, are incorporated herein by reference, and the Sections hereafter referred to are Sections of the Research Disclosure.

The silver halide emulsions employed in the elements of this invention can be either negative-working or positive-working. Suitable emulsions and their preparation as well as methods of chemical and spectral sensitization are described in Sections I through IV. Color materials and development modifiers are described in Sections V and XXI. Vehicles are described in Section IX, and various additives such as brighteners, antifogging agents, stabilizers, light absorbing and scattering materials, hardeners, coating aids, plasticizers, lubricants and 60 matting agents are described, for example, in Sections V, VI, VIII, X, XI, XII, and XVI. Manufacturing methods are described in Sections XIV and XV, other layers and supports in Sections XIII and XVII, processing methods and agents in Sections XIX and XX, and exposure alternatives in Section XVIII.

The invention materials herein may be used in combination with photographic compounds such as those based on 3-acylamino- and 3-anilino-5-pyrazolones

(other than those of the invention) and heterocyclic couplers (e.g. pyrazoloazoles) such as those described in EP 285,274; U.S. Pat. No. 4,540,654; EP 119,860, which may contain different ballasts or coupling-off groups such as those described in U.S. Pat. Nos. 4,301,235; 4,853,319 and 4,351,897. They may also be used in association with yellow or cyan colored couplers (e.g. to adjust levels of interlayer correction) and, in color-negative applications, with masking couplers such as those described in EP 213,490; Japanese Published Application 58-172,647; U.S. Pat. No. 2,983,608; German Application DE 2,706,117C; U.K. Patent 1,530,272; Japanese Application A-113935; U.S. Pat. No. 4,070,191 and 4,273,861; and German Application DE 2,643,965. The masking couplers may be shifted or blocked.

With regard to the inclusion of other couplers in the element, the presence of certain coupling-off groups is well known in the art. Such groups can determine the chemical equivalency of the coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction and the like.

The presence of hydrogen at the coupling site provides a 4-equivalent coupler, and the presence of another coupling-off group provides a 2-equivalent coupler. Representative classes of such coupling-off groups include, for example, chloro, alkoxy, aryloxy, hetero-oxo, sulfonyloxy, acyloxy, acyl, heterocycl, sulfonamido, mercaptotetrazole, benzothiazole, mercaptopro-30

pic acid, phosphonyloxy, arylthio, and arylazo. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in U.K. Patent and published application Nos. 1,466,728, 1,531,927, 1,533,039, 2,006,755A and 2,017,704A, the disclosures of which are incorporated herein by reference.

The invention materials may also be used in association with materials that accelerate or otherwise modify the processing steps e.g. of bleaching or fixing to improve the quality of the image. Bleach accelerators described in EP 193,389; EP 301,477; U.S. Pat. Nos. 4,163,669; 4,865,956; and 4,923,784 are particularly useful. Also contemplated is use of the compositions in association with nucleating agents, development accelerators or their precursors (UK Patent 2,097,140; U.K. Patent 2,131,188); electron transfer agents (U.S. Pat. No. 4,859,578; 4,912,025); antifogging and anti color-mixing agents such as derivatives of hydroquinones, aminophenols, amines, gallic acid; catechol; ascorbic acid; hydrazides; sulfonamidophenols; and non color-forming couplers.

The invention materials may also be used in combination with filter dye layers comprising colloidal silver sol or yellow, cyan, and/or magenta filter dyes, either as oil-in-water dispersions, latex dispersions or as solid particle dispersions. Additionally, they may be used with "smearing" couplers (e.g. as described in U.S. Pat. No. 4,366,237; EP 96,570; U.S. Pat. Nos. 4,420,556; and 4,543,323.) Also, the compositions may be blocked or coated in protected form as described, for example, in

Japanese Application 61/258,249 or U.S. Pat. No. 5,019,492.

The invention materials may further be used in combination with image-modifying compounds such as "Developer Inhibitor-Releasing" compounds (DIR's). DIR's useful in conjunction with the materials of the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 72,573; 335,319; 336,411; 346, 899; 362, 870; 365,252; 65,346; 373,382; 376,212; 377,463; 378,236; 384,670; 96,486; 401,612; 401,613.

Such compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptothiazoles, mercaptotriazoles, mercaptooxadiazoles, mercaptodiazoles, mercaptooxathiazoles, telleurotetrazoles or benzodiazoles. In a preferred embodiment, the inhibitor moiety or group is selected from the following formulas:



wherein  $R_I$  is selected from the group consisting of straight and branched alkyls and alkoxy typically of from 1 to about 8 carbon atoms, benzyl and phenyl groups and said groups containing none, one, or more than one such substituent;  $R_{II}$  is selected from  $R_I$  and  $-SR_I$ ;  $R_{III}$  is a straight or branched alkyl group of from 1 to about 5 carbon atoms and  $m$  is from 1 to 3; and  $R_{IV}$  is selected from the group consisting of hydrogen, halogens and alkoxy, phenyl and carbonamido groups,  $-COOR_V$  and  $-NHCOOR_V$  wherein  $R_V$  is selected from substituted and unsubstituted alkyl and aryl groups. 10

Although it is typical that the coupler moiety included in the developer inhibitor-releasing coupler forms an image dye corresponding to the layer in which it is located, it may also form a different color as one associated with a different film layer. It may also be useful that the coupler moiety included in the developer inhibitor-releasing coupler forms colorless products and/or products that wash out of the photographic material during processing (so-called "universal" couplers). 15

As mentioned, the developer inhibitor-releasing coupler may include a timing group which produces the time-delayed release of the inhibitor group such as groups utilizing the cleavage reaction of a hemiacetal (U.S. Pat. No. 4,146,396, Japanese Applications 60-249148; 60-249149); groups using an intramolecular nucleophilic substitution reaction (U.S. Pat. No. 4,248,962); groups utilizing an electron transfer reaction along a conjugated system (U.S. Pat. Nos. 4,409,323; 4,421,845; Japanese Applications 57-188035; 58-98728; 25

58-209736; 58-209738) groups utilizing ester hydrolysis (German Patent Application (OLS) No. 2,626,315; groups utilizing the cleavage of imino ketals (U.S. Pat. No. 4,546,073); groups that function as a coupler or reducing agent after the coupler reaction (U.S. Pat. Nos. 4,438,193; 4,618,571) and groups that combine the features described above. It is typical that the timing group or moiety is of one of the formulas:



wherein IN is the inhibitor moiety, Z is selected from the group consisting of nitro, cyano, alkylsulfonyl; sulfamoyl ( $-SO_2NR_2$ ); and sulfonamido ( $-NRSO_2R$ ) groups; n is 0 or 1; and  $R_V$  is selected from the group consisting of substituted and unsubstituted alkyl and phenyl groups. The oxygen atom of each timing group is bonded to the coupling-off position of the respective coupler moiety of the DIAR.

Suitable developer inhibitor-releasing couplers for use in the present invention include, but are not limited to, the following:



-continued



-continued



D7



D8

It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire PO101 7DQ, England, incorporated herein by reference. Materials of the invention may be coated on pH adjusted support as described in U.S. Pat. No. 4,917,994; with epoxy solvents (EP 0 64 961); with nickel complex stabilizers (U.S. Pat. Nos. 4,346,165; 4,540,653 and 4,906,559 for example); with ballasted chelating agents such as those in U.S. Pat. No. 4,994,359 to reduce sensitivity to polyvalent cations such as calcium; and with stain reducing compounds such as described in U.S. Pat. Nos. 5,068,171 and 5,096,805. Other compounds useful in combination with the invention are disclosed in Japanese Published Applications having the following Derwent Abstract Accession Numbers: 83-0 9,959; 83-62,586; 90-072,629, 90-072,630; 90-072,632; 90-072,633; 90-072,634; 90-077,822; 90-078,229; 90-078,230; 90-079,336; 90-079,338; 90-079,690; 90-079,691; 90-080,487; 90-080,489; 90-080,490; 90-080,491; 90-080,492; 90-080,494; 90-085,928; 90-086,669; 90-086,670; 90-087,361; 90-087,362; 90-087,363; 90-087,364; 90-088,096; 90-088,097; 90-093,662; 90-093,663; 90-093,664; 90-093,665; 90-093,666; 90-093,668; 90-94,055; 90-094,056; 90-101,937; 90-103,409; 90-51,577.

Especially useful in this invention are tabular grain silver halide emulsions. Specifically contemplated tabular grain emulsions are those in which greater than 50 percent of the total projected area of the emulsion grains are accounted for by tabular grains having a

40

45

thickness of less than 0.3 micron (0.5 micron for blue sensitive emulsion) and an average tabularity (T) of greater than 25 (preferably greater than 100), where the term "tabularity" is employed in its art recognized usage as

$$T = ECD/t^2$$

where

ECD is the average equivalent circular diameter of the tabular grains in micrometers and

$t$  is the average thickness in micrometers of the tabular grains.

The average useful ECD of photographic emulsions can range up to about 10 micrometers, although in practice emulsion ECD's seldom exceed about 4 micrometers. Since both photographic speed and granularity increase with increasing ECD's, it is generally preferred to employ the smallest tabular grain ECD's compatible with achieving aim speed requirements.

Emulsion tabularity increases markedly with reductions in tabular grain thickness. It is generally preferred that aim tabular grain projected areas be satisfied by thin ( $t < 0.2$  micrometers) tabular grains. To achieve the lowest levels of granularity it is preferred that aim tabular grain projected areas be satisfied with ultrathin ( $t < 0.06$  micrometers) tabular grains. Tabular grain thicknesses typically range down to about 0.02 micrometers. However, still lower tabular grain thicknesses are contemplated. For example, Daubendiek et al U.S. Pat. No. 4,672,027 reports a 3 mole percent iodide tabular

grain silver bromoiodide emulsion having a grain thickness of 0,017 micrometers.

As noted above tabular grains of less than the specified thickness account for at least 50 percent of the total grain projected area of the emulsion. To maximize the advantages of high tabularity it is generally preferred that tabular grains satisfying the stated thickness criterion account for the highest conveniently attainable percentage of the total grain projected area of the emulsion. For example, in preferred emulsions, tabular grains satisfying the stated thickness criteria above account for at least 70 percent of the total grain projected area. In the highest performance tabular grain emulsions, tabular grains satisfying the thickness criteria above account for at least 90 percent of total grain projected area. 10

Suitable tabular grain emulsions can be selected from among a variety of conventional teachings, such as those of the following: Research Disclosure, Item 22534, January 1983, published by Kenneth Mason Publications, Ltd., Emsworth, Hampshire PO10 7DD, England; U.S. Pat. Nos. 4,439,520; 4,414,310; 4,433,048; 4,643,966; 4,647,528; 4,665,012; 4,672,027; 4,678,745; 4,693,964; 4,713,320; 4,722,886; 4,755,456; 4,775,617; 4,797,354; 4,801,522; 4,806,461; 4,835,095; 4,853,322; 4,914,014; 4,962,015; 4,985,350; 5,061,069 and 5,061,616. 20

The emulsions can be surface-sensitive emulsions, i.e., emulsions that form latent images primarily on the surfaces of the silver halide grains, or internal latent images predominantly in-the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent. 30

Photographic elements can be exposed to actinic radiation, typically in the visible region of the spectrum, to form a latent image and can then be processed to form a visible dye image. Processing to form a visible dye image includes the step of contacting the element with a color developing agent to reduce developable silver halide and oxidize the color developing agent. Oxidized color developing agent in turn reacts with the coupler to yield a dye. 40

With negative-working silver halide, the processing step described above provides a negative image. The described elements can be processed in the known C-41 color process as described in The British Journal of Photography Annual of 1988, pages 191-198. The described elements are optionally processed in the known color processes for processing color print papers, such as the known RA-4 process of Eastman Kodak Company and as described in the British Journal of Photography Annual of 1988, pages 198-199. To provide a positive (or reversal) image, the color development step can be preceded by development with a non-chromogenic developing agent to develop exposed silver halide, but not form dye, followed by uniformly fogging the element to render unexposed silver halide developable. Alternatively, a direct positive emulsion can be employed to obtain a positive image. 50

Preferred color developing agents are p-phenylenediamines. Especially preferred are: 4-amino-N,N-diethylaniline hydrochloride, 4-amino-3-methyl-N,N-diethylaniline hydrochloride, 4-amino-3-methyl-N-ethyl-N-( $\beta$ -(methanesulfonamido)ethyl)aniline sesquisulfate hydrate, 60

4-amino-3-methyl-N-ethyl-N-( $\beta$ -hydroxyethyl)aniline sulfate,

4-amino-3- $\beta$ -(methanesulfonamido)ethyl-N,N-diethylaniline hydrochloride and

4-amino-N-ethyl-N-(2-methoxyethyl)-m-toluidine di-p-toluene sulfonic acid.

Development is usually followed by the conventional steps of bleaching, fixing, or bleach-fixing, to remove silver or silver halide, washing, and drying.

15 It is understood throughout this specification and claims that any reference to a substituent by the identification of a group containing a substitutable hydrogen (e.g. alkyl, amine, aryl, alkoxy, heterocyclic, etc.), unless otherwise specifically stated, shall encompass not only the substituent's unsubstituted form, but also its form substituted with any photographically useful substituents. Usually the substituent will have less than 30 carbon atoms and typically less than 20 carbon atoms. 25

#### SYNTHETIC EXAMPLE

The following Scheme A outlines a method for the preparation of a coupler of the invention:

#### SYTHETIC SCHEME A



SYNTHETIC SCHEME A  
-continued

## Preparation of Ethyl-3-ethoxy-3-iminopropionate hydrochloride

Hydrogen chloride gas was bubbled through a stirred solution of ethyl cyanoacetate (900 g, 7.96 moles), ethanol (410 ml, 7.0 moles) and diethyl ether (2.4 liters). The temperature was kept at <15° C. by use of a cooling bath. After 3.5 hours 395 g (10.8 moles) of HCl had been absorbed. The flask was kept in the cold room over the weekend. The crystalline white product was filtered off, washed with diethyl ether, then petroleum ether and dried under vacuum. The yield was 1210 g (88%).

Preparation of Ethyl-3,3,3-trimethoxypropionate Ethyl-3-ethoxy-3-iminopropionate hydrochloride (1.21 kg, 6.19 moles) was stirred with methanol (3 liters) at room temperature overnight. The precipitated ammonium chloride was filtered off and most of the methanol was removed on the rotavapor. The residue was treated with diethyl ether (1.5 liters) and washed with water (1.5 liters) followed by 2×1.5 liters of 10% sodium carbonate solution. The first sodium carbonate wash removed some yellow color. The ether layer was separated, dried ( $MgSO_4$ ) and the solvent removed on the rotavapor to give a colorless liquid. The yield was 867 g (73%). The structure of the product was confirmed by NMR and IR spectroscopy.

## Preparation of Pyrazolone A

A mixture of ethyl-3,3,3-trimethoxypropionate (35 g, 0.18 moles), 2-chloro-4-dodecylsulphonylaniline (54 g, 0.15 moles), p-toluenesulphonic acid (0.3 g) and toluene (300 ml) was stirred and heated. When the temperature had reached 60° C., concentrated sulphuric acid (18 drops) was added. When the temperature reached 70° C., solvent started to distil over. The temperature of distillation rose from 70° C. to 112° C. Heating was continued at 112° C for 15 minutes when 150 ml of solvent had distilled over. TLC showed about 10% of starting aniline was still present. A further 3 g of the orthoester and 0.2 g of p-toluenesulphonic acid were added along with more toluene (200 ml). Heating was continued for 20 minutes while distilling another 100 ml of solvent. TLC now showed a major spot with only a trace of the starting aniline. The solvent was removed on the rotavapor to give an oil (81 g). This was dissolved in acetic acid (230 ml) and 2,4,6-trichlorophenylhydrazine (30.67 g, 0.145 moles) was added. The resultant slurry was stirred at room temperature. After 2 hours a solution was obtained. The reaction mixture was stirred overnight at room temperature until it had set solid. It was transferred to a rotavapor flask using

warm petroleum ether and the solvents removed to give a red oil (133 g). This oil was transferred to a 3-necked flask using methanol (380 ml) and a solution of potassium hydroxide (42 g, 0.75 moles) in methanol (230 ml)

5 added with good stirring and ice-bath cooling over 10 minutes at >20° C. The resultant dark red solution was stirred at 15°–20° C. for 10 minutes and then acetic acid (44 ml) was added. The precipitated oil soon crystallized. The mixture was stirred at room temperature for 10 hours and the solid filtered off, washed with methanol and then recrystallized from acetic acid (280 ml). When the hot acetic acid solution had cooled to 35° C., methanol (550 ml) was added, the mixture stirred at 10° C. for 1 hour, filtered, washed with methanol and dried.

15 The yield was 65.1 g (72.3%). Hplc-100%.

Calc. C, 51.85; H, 5.50; Cl, 22.97; N, 6.69; S, 5.09. Found C, 52.18; H, 5.35; Cl, 22.82; N, 6.76; S, 5.16.

## Preparation of 4-Acetamido-benzenesulphonic acid

To 4-acetamidobenzenesulphonyl chloride (400 g, 1.72 moles) was added with stirring a solution of sodium sulphite (431.7 g, 3.42 moles) in water (2 liters). A solution of 50% sodium hydroxide (240 ml) was added dropwise over 35 minutes using a cooling bath to keep the temperature below 30° C. The pH was thus maintained in the range 6.5–7.0. The mixture was stirred at room temperature for 2 hours and acidified by adding conc. sulphuric acid (170 ml) with ice-bath cooling. The precipitated white solid was filtered off, washed with water and dried at 50° C. The yield was 324.2 g (94%). This was used in the next stage without further purification.

## Preparation of 4-Dodecylsulphonylacetanilide

To 4-acetamidobenzenesulphonic acid (324 g, 1.63 moles) and dimethylformamide (1.6 liters) was added in portions with stirring anhydrous potassium carbonate (337 g, 244 moles) followed by 1-bromododecane (472 g, 1.88 moles). The mixture was stirred and heated at 100° C. for 6 hours. It was cooled to room temperature, poured into 5 liters of water, stirred for 30 minutes, the white solid filtered off, washed with water and pulled dry. It was recrystallized from methanol (2 liters) to give 521.7 g (87%) of pure product.

Calc. C, 65.4; H, 8.99; N, 3.81; S, 8.72. Found C, 65.16; H, 8.58; N, 3.82; S, 8.49.

## Preparation of 4-Dodecylsulphonylaniline

A mixture of 4-dodecylsulphonylacetanilide (594 g, 1.62 moles) and dioxane (2.3 liters) was stirred and heated to 70° C. (solution). Conc. HCl (3450 ml) was added over 5 minutes and heating continued. After a few minutes a white solid had precipitated. The mixture was stirred at reflux for 2 hours. At first there was a tendency for the mixture to foam excessively so that the heating mantle had to be removed for a time to control the foaming. The mixture was cooled to room temperature and added to stirred ice-water (5 liters) containing sodium hydroxide (200 g). The product was filtered off, washed with water and dried. The yield was 520 g (99%).

Calc. C, 66.42; H, 9.609; N, 4.30; X, 9.85. Found C, 66.25; H, 9.22; N, 4.26; X, 9.46.

## Preparation of 2-Chloro-4-dodecylsulphonylaniline

A mixture of 4-dodecylsulphonylaniline (519.8 g, 1.6 moles), 1,2-dichlorethane (2.5 liters) and N-chlorosuccinimide (NCS) (110 g, 0.825 moles) was stirred at reflux for 45 minutes, then a further 60 g (0.45 moles) of NCS added. Refluxing was continued for another 45 minutes and another 53 g of NCS was added. The mix-

ture was refluxed for another hour. The total amount of NCS used was 223 g (1.67 moles). TLC showed no starting material. The solvent was removed on the rotavapor, the residue dissolved in ethyl acetate (2 liters), washed with 3×1.5 liters of hot water, dried (MgSO<sub>4</sub>) and the solvent removed. The product was recrystallized twice from petroleum ether plus a little ethyl acetate to give 513.6 g (89%).

Calc. C, 60.06; H, 8.40; Cl, 9.85; N, 3.89; X, 8.91. Found C, 59.88; H, 7.96; Cl, 9.91; N, 3.86; S, 8.59.

Preparation of bis-4,4'-undecylcarbonamidophenyl disulfide

A solution of lauroyl chloride (48.8 g, 0.21 mole) in THF (100 ml) was added to a solution of 4-aminophenyl disulfide (24.8 g, 0.1 mole) in THF (100 ml) and pyrdine (80 ml) at 20° C. over ½ hour. A thick precipitate was formed. The suspension was stirred at room temperature for ¾ hour and then added to cold 10% hydrochloric acid (1500 ml). The solid was collected by filtration and washed well with water. The product, a grey colored solid, gave 61.1 g (100%).

Elemental Analysis Requires C, 70.54; H, 9.21; N, 4.57; S, 10.46. Found C, 70.66; H, 9.29; N, 4.48; S, 9.75 15 70.61; 9.57; 4.46

#### Preparation of Coupler I-2

Sulphuryl chloride (2.8 g, 21 mmole) was added to a suspension of bis-4,4'-undecylcarbonamidophenyl disulfide (12.9 g, 21 m mole) in dichloromethane (175 ml) and stirred at room temperature for 1.5 hours. The volatiles were removed by rotary evaporation below 30 40° C. A solution of pyrazolone A (21.7 g, 35 m mole) in DMF (50 ml) was added rapidly to the solid and stirring at room temperature continued for 75 hours. The suspension was slowly poured into 3N hydrochloric acid (750 ml) and the resulting aqueous phase decanted off. The residue was dissolved in ethyl acetate (500 ml) and the organic solution washed with water (2×100 ml), dried, and evaporated under reduced pressure. The crude material was crystallized from ethyl acetate (50 ml)/60-80 pet ether (200 ml) to give the 40 product, as a white solid, 22.8 g (70%).

Elemental Analysis Requires C, 58.31; H, 6.53; Cl, 15.30; N, 6.05; S, 6.92. Found C, 58.36; H, 6.51; Cl, 15.58; N, 6.00; S, 6.83. 58.50 6.48 6.03

#### Photographic Examples

The following Tables illustrate the advantages of the invention. The formulas for the couplers used are shown following the examples. For the samples of Table I, photographic elements were prepared by coating a cellulose acetate-butylate film support (with a rem-jet antihalation backing) with a photosensitive layer containing a silver bromoiodide emulsion at 1.08 g/m<sup>2</sup>, gelatin at 3.77 g/m<sup>2</sup> and an image coupler dispersed in the coupler/addenda as indicated at 0.52 55 mmoles/m<sup>2</sup>. The photosensitive layer was overcoated with a layer containing gelatin at 2.69 g/m<sup>2</sup> and bis-

vinylsulfonyl methyl ether hardner at 1.75 weight percent based on total gel.

For the samples of Table II, photographic elements were prepared by coating a cellulose acetate film support with a photosensitive layer containing a green-sensitized silver bromoiodide emulsion at 1.61 g/m<sup>2</sup>, gelatin at 2.42 g/m<sup>2</sup> and an image coupler dispersed in its own weight of solvent at 1.04 mmoles/m<sup>2</sup> with bis-(vinylsulphonyl)methane at 0.06 g/m<sup>2</sup>. The photosensitive layer was overcoated with a layer containing gelatin at 1.5 g/m<sup>2</sup> and bis-vinylsulfonyl methyl ether hardner at 1.75 weight percent based on total gel.

Samples of each element were exposed imagewise through a stepped density test object and subjected to the Kodak Flexicolor C-41 process as described in *British Journal of Photography Annual*, 1988, pp. 196-198. The coupler dispersion was as shown in the tables for solvent and stabilizer.

Thus treated samples were then subjected to tests to evaluate the photographic properties of the elements as follows:

“Delta Dmin” was determined by subtracting the minimum density when a 1% sulfuric acid stop bath is utilized after the development process from the minimum density obtained when no stop bath was employed. This result is a measure of continued coupling which causes an undesired nonimagewise stain. Lower numbers are better since that indicates less stain resulting in the standard unstopped process.

“Developed Silver” was determined by measuring the amount of silver developed at midscale exposure using X-ray fluorescence. If the released thiol has adverse interactions with the silver it will be reflected in the amount of developed silver.

“Delta Dmax” was determined by subtracting the green density corresponding to maximum exposure measured immediately after processing from the value obtained when the sample is stored at 38 degrees C. and 50% relative humidity for 24 hours before measuring the density. The increase in maximum density is a measure of the extent to which the element contains a semi-stable leuco dye which does not convert to a visible dye until after development. This is undesirable since the printer cannot adjust for the unpredictability of this phenomenon. Lower numbers are more desirable for this measurement since that indicates less leuco dye formation.

“Coupler/Solvent/Stabilizer” indicates the mol ratio of these components and identifies the solvent used. 50 CS-1 is N,N-dibutyl lauramide and CS-2 is tricresyl phosphate. The stabilizer is N,N-di-n-butyl-2-n-butoxy-5-(1,1,3,3-tetramethylbutyl)aniline.

$\lambda_{max}$  signifies the wavelength of maximum light absorption in nanometers (nm) and HBW, shown parenthetically, shows the half-band width.

In the tables, inventive and comparison samples are grouped for ready comparison.

TABLE I

| Sample | Coupler | Type | Delta Dmin | Developed Silver | Delta Dmax | Mol Ratio Coupler/Solvent/Stabilizer | $\lambda_{max}$ (nm) (HRW) |
|--------|---------|------|------------|------------------|------------|--------------------------------------|----------------------------|
| 1      | C-1     | Comp | 0.074      | 29.6             | +0.009     | 1:8:2 (CS-1)                         | 544 (81)                   |
| 2      | I-1     | Inv  | 0.027      | 31.1             | +0.003     | 1:8:2 (CS-1)                         | 545 (81)                   |
| 3      | C-2     | Comp | 0.039      | 29.5             | +0.024     | 1:8:2 (CS-1)                         | 546 (83)                   |
| 4      | I-2     | Inv  | 0.020      | 29.9             | +0.007     | 1:8:2 (CS-1)                         | 546 (82)                   |
| 5      | C-3     | Comp | 0.144      | 33.8             | +0.052     | 1:1:0 (CS-2)                         | 543 (84)                   |
| 6      | I-3     | Inv  | 0.053      | 29.6             | +0.021     | 1:1:0 (CS-2)                         | 544 (83)                   |

TABLE II

| Sample | Coupler | Type | Delta Dmin | Delta Dmax | Coupler/Solvent/Stabilizer | $\lambda_{max}$ (nm) | 5  |
|--------|---------|------|------------|------------|----------------------------|----------------------|----|
| 7      | C-1     | Comp | 0.48       | +0.72      | 1:1:0(CS-2)                | 547 (84)             |    |
| 8      | I-4     | Inv  | 0.48       | +0.24      | 1:1:0(CS-2)                | 548 (88.5)           | 10 |
| 9      | I-5     | Inv  | 0.38       | +0.15      | 1:1:0(CS-2)                | 551 (82)             |    |
| 10     | C-2     | Comp | 0.57       | +0.14      | 1:1:0(CS-2)                | 549 (83)             |    |
| 11     | I-6     | Inv  | 0.24       | +0.14      | 1:1:0(CS-2)                | 548 (84)             | 15 |

The data summarized in the tables shows the advantages of the invention. A comparison of the results for the invention couplers versus the comparison couplers of Table I shows that the invention provides less fogging or staining (lower Dmin values for the invention); less semi-stable leuco dye formation (lower Delta Dmax values); and equal or better hue (longer  $\lambda_{max}$  and narrower half-band width.)

The amount of developed silver appears equivalent. Similar results are demonstrated in Table II.

-continued

I-3



I-4



I-5



-continued



The invention has been described in detail with particular reference to preferred embodiments thereof, but it will be understood that the invention includes varia-

tions and modifications within the spirit and scope of the invention.

What is claimed is:

1. A photographic element comprising a light-sensitive silver halide layer having associated therewith a coupler which is a pyrazolone compound containing a parent having a phenyl and an anilino substituent and a coupling-off group at the 4-position, the coupler having the formula:



wherein:

at least one  $R^a$  is located in the 4-position of the anilino ring and is a substituent selected from those which are attached to the anilino ring by a member selected from the group consisting of  $-SO_2-$ ;  $-SO_2-$ ;  $-OSO_2-$ ;  $-SO_2N<$ ;  $>NSO_2-$ ;  $-CON<$ ;  $-CO-$ ;  $-OCO-$ ;  $-COO-$ ;  $-CN$ ;  $-NO_2$ ; and  $-CF_3$ ;

each  $R^c$  is individually halogen, or substituted or unsubstituted alkyl, aryloxy or alkoxy;

each  $R^b$  is individually hydrogen or a substituent selected so that the sum of the Hammett sigma values for all  $R^a$ ,  $R^b$ , and  $R^c$  groups is at least 1.1 and the combination of such substituents is sufficient to ballast the dye formed by the parent upon coupling;

$q$  is 0 to 3, and  $r$  is 0 to 2;  $R^2$  is hydrogen or alkyl of up to two carbon atoms; each  $R^3$  is independently a substituent;  $R^4$  is a substituted or unsubstituted alkyl or aryl group;  $R^5$  is hydrogen or substituted or unsubstituted alkyl;  $p$  is 0 to 3;

provided that any combination of  $R^3$ ,  $R^4$ , and  $R^5$  may join together to form a ring; and

provided further that each of  $R^2$  through  $R^5$  are selected such that the calculated log P of the thiophenol corresponding to the substituent at the 4-position of the pyrazolone is at least 4.

2. The element of claim 1 wherein the calculated log P value is at least 4.5.

3. The element of claim 1 wherein the calculated log P value is at least 5.0.

4. The element of claim 1 wherein at least two  $R^c$  on the 1-phenyl ring are chlorine, and  $R^c$  on the anilino ring is chlorine.

5. The element of claim 1 wherein  $R^a$  is an unsubstituted alkylsulfonyl group in which the alkyl group contains 2 to 30 carbon atoms.

6. The element of claim 1 wherein  $R^a$  includes a ballast group.

7. A process of forming an image comprising contacting an exposed element as described in claim 1 with a color developing chemical.

8. The process of claim 7 wherein the color developing chemical is a para-phenylenediamine.

\* \* \* \* \*